

Aug. 20, 1940.

A. BECK

2,212,413

RUG

Filed March 13, 1939

*Fig. 1*



*Inventor:*  
August Beck  
*By* *Dammer Dommer*  
*Attorneys.*

## UNITED STATES PATENT OFFICE

2,212,413

## RUG

August Beck, Oshkosh, Wis., assignor to Waite Carpet Company, Oshkosh, Wis., a corporation of Wisconsin

Application March 13, 1939, Serial No. 261,473

3 Claims. (Cl. 139—420)

Efforts have been made in the past to make use of sisal as a constituent in rug weaving, but difficulties have been encountered by reason of the stiff wiry character of the filaments, which resist packing or copression and make it difficult to beat up the sisal strands in the loom, so that, unless the fiber strands are firmly and permanently anchored in place, the rug will be sleazy or loose-textured and will not maintain its shape.

Sisal possesses certain very desirable qualities, however, principally by reason of its bright lustrous appearance and its ability to take permanent dyes, so that the use of small quantities of sisal has heretofore been attempted for the purpose of brightening the appearance of the rug, and maintaining an apparent newness or freshness even after the dull and less permanently dyed materials have faded. Such use of sisal in the past, however, has been limited mainly to narrow warp stripes which were closely compacted by the proximity of the more compressible materials so that it was possible to hold the sisal warp stripes in position. I have found, however, that highly satisfactory results can be secured by the use of a sisal woof or filler in conjunction with a fiber warp, by which means a warp in which the strands are composed of twisted paper known in the art as fiber.

The fiber, however, is of a much duller color tone and colored with relatively impermanent dyes as compared with the lustrous tones of the sisal which serves to brighten the rug and give it a permanent luster, so that the fading of the fiber will not unduly impair the appearance of the rug, which will thus maintain its freshness for a long period of time.

Further objects and details will appear from a description of the invention in conjunction with the accompanying drawing, wherein—

Figure 1 is a section of a rug displaying the characteristics of the present invention; and

Fig. 2 is a sectional view taken on line 2—2 of Fig. 1.

The rug consists of woof strands A of permanently colored sisal of relatively heavy bulk as compared with the warp strands B of fiber twine of relatively duller color tones and dyed with relatively impermanent dyes as compared with the dying of the sisal.

The contiguous woof strands are united by the bends of loops C at the edges of the rug, so that the woof strands are practically continuous throughout substantial areas of the rug, and the outwardly presented loops serve to afford the finished side edges of the rug. The individual

warp strands are of much smaller bulk than the woof strands and are arranged in pairs, each pair being looped over two woof strands and under the next two, and the pairs of warp strands are twill woven so as to give a diagonally ribbed effect throughout the rug.

As shown, the entire woof of the rug is composed of the bulky sisal strands and the entire warp of the less bulky fiber strands, with the exception of one or more warp stripes D of sisal which as shown are of equal bulk with the sisal strands in the woof. The use of occasional sisal warp strands intersecting the sisal woof strands is permissible in limited degree where the number of adjacent warp strands is very limited, as for instance two or possibly three warp strands, so that the areas of intersection of the sisal strands (warp and woof) are so reduced as to hold the sisal permanently anchored against displacement by the compacting influence of the adjacent fiber, which latter is a readily compactible substance which serves admirably for the purpose of holding the sisal strands in place.

As before stated, the fiber warp is dyed with relatively impermanent dyes, which affords a somewhat dull or non-lustrous color tone in marked contrast to the lustrous silvery appearance of the natural sisal, or the lustrous color tones imparted by dyeing with permanent dyes, so that, by employing a filler of relatively bulky sisal strands, large areas of the sisal are exposed in the completed rug which thus displays the lustrous coloration of the sisal and compensates against the duller tones of the fiber, or the tendency of the latter to fade after a period of use.

By employing the sisal exclusively in the woof of the rug, with the possible exception of narrow warp stripes, the sisal strands will lie in adjacent relation to one another throughout all, or practically all, of the entire area, so that there will be no areas of intersection, except possibly the limited areas where narrow sisal warp stripes are used for pattern effect or otherwise, with the result that the strands composing the sisal woof will be firmly and permanently anchored by the compactible fiber warp, so that a closely textured and firmly interwoven rug will be provided which secures the advantages of a large display of sisal without permitting the sisal strands to escape the close confinement necessary in order to prevent warping or stretching of the rug.

Furthermore, the sisal affords a strong, re-

silent or springy woof by reason of the wiry character of the sisal filaments composing the woof strands, so that the rug will not tend to mat down in use, but will maintain a springy 5 resilient texture for an indefinite period of time, and at the same time the compressible resilient character of the bulky sisal woof affords a backing for the exposed fiber warp, which guards the latter against abrasive action, which is highly desirable, since the latter, unless protected by a 10 resilient backing, would be subject to deterioration through abrasive action.

The combination of sisal and fiber here described has proved to be highly satisfactory in 15 commercial use, both by reason of the striking appearance of the rug and by reason of its durable and resistant qualities, as well as by its freedom from warping due to displacement of the sisal strands.

20 I claim:

1. A rug composed throughout substantially 25 its entire area of closely lying parallel woof strands of lustrous sisal and warp strands of dull toned fiber, the fiber warp strands being interwoven with the sisal woof strands and closely compacted to anchor the woof strands against displacement, the sisal strands being dyed at least in part with relatively permanent dyes and displaying a lustrous coloration, and the

fiber strands being dyed in relatively impermanent dyes and displaying a duller coloration.

2. A rug composed throughout substantially 5 its entire area of closely lying parallel woof strands of relatively less bulky sisal and warp strands of relatively less bulky fiber, the fiber warp strands being interwoven with the sisal woof strands and closely compacted to anchor the woof strands against displacement, the sisal strands being dyed at least in part with relatively 10 permanent dyes and displaying a lustrous coloration, and the fiber strands being dyed in relatively impermanent dyes and displaying a duller coloration.

3. A rug consisting throughout substantially 15 its entire area of bulky woof strands of permanently colored lustrous sisal lying in close parallel relation and connected by looping at the side edges of the rug, the woof strands being permanently anchored in place by warp strands interwoven with the woof strands and closely compacted to permanently anchor the sisal woof strands against displacement, the individual warp strands being of lesser bulk than the sisal 20 woof strands and dyed in relatively impermanent 25 dyes, and presenting a relatively dull coloration as contrasted with the lustrous coloration of the sisal.

AUGUST BECK.